

## UNITED STATES PATENT OFFICE.

ROGER MAGONDEAUX, OF PARIS, FRANCE.

## PROCESS FOR THE MANUFACTURE OF GRANULAR CELLULOSE.

No Drawing. Application filed November 18, 1924, Serial No. 750,716, and in France November 20, 1923.

It is known that compressed or dissolved explosive or inflammable gases and explosive or inflammable liquids, can only be stored without danger when absorbed in a porous material with which the container is faced. Under these conditions, there may be a certain pressure within the container which yet is safe for transport.

This is especially the case with dissolved acetylene.

Various porous materials have been proposed for this purpose; their function has become particularly onerous when flasks of dissolved gas are placed on motor vehicles where the facing is subject to shock, to vibration, and also to differences of temperature; so much is this the case that minute regulations have been drawn up respecting them, especially as regards the percentage of porosity which the material should possess, and as regards the capacity of the material of becoming rammed, which capacity must not be exceeded in spite of most violent blows.

Among the materials proposed are sawdust, the pith of the elder tree, etc., but in the form of these two varieties, cellulose does not fulfill the conditions of porosity and unalterableness.

This invention relates to a process for treating sawdust which transforms and gives to it the required qualities; the invention relates also to the new commercial product resulting from the treatment, which product really consists of calibrated porous granules of cellulose.

Sawdust is first sieved through two sieves, the larger mesh sieve excluding too large pieces such as chips or pieces, while the fine mesh sieve excludes dust in a too fine state of division.

It is then subject to a treatment with soda lye, for example, having for its object, and should have for result, to remove incrusting matters such as lignines and lignones of the wood, and to leave only lignocellulose. This is really the first operation in the manu-

facture of paper pulp. It should therefore be understood that the treatment may be any one of the known treatments with soda, bisulphite, etc., in a boiler or autoclave, according to the conditions of working and the material employed.

Pure cellulose in the form of light porous homogeneous granules, not attacked by acetone, is the result of such operation.

The cellulose granules are treated in a centrifugal machine and dried, after which they are in a state suitable for storing dissolved gases. The porosity of the granules approaches 70%, or rather less, and they are very light.

They can be placed in containers under direct ramming, and by tamping in give an absolutely equal distribution without "heaving." A kilogram may fill a 3 litre vessel, and receive 500 litres of dissolved gas, leaving all freedom of expansion, but preventing spitting which is very dangerous, not only by the restraint it brings to the outlet of the gas, but above all, by the diminution of volume and the pockets resulting therefrom.

The cellulose granules may be employed for other purposes than facing flasks of dissolved acetylene which is given by way of illustration only.

Having now particularly described and ascertained the nature of my said invention and in what manner the same is to be performed, I declare that what I claim is:

The process, for the object specified, of treating sawdust, which consists in passing the same through sieves of predetermined mesh to obtain a particular uniform size of granule depending upon the purpose for which it is desired, and sifting such graded sawdust to remove dust, then subjecting the granules to treatment in an alkaline solution, and finally centrifuging and drying the granular product lastly obtained.

In testimony whereof I affix my signature.

ROGER MAGONDEAUX,